

## UNITED STATES PATENT OFFICE

2,221,245

## MAGNESIUM BASE ALLOY

Joseph D. Hanawalt and John C. McDonald, Midland, Mich., assignors to The Dow Chemical Company, Midland, Mich., a corporation of Michigan

No Drawing. Application November 13, 1939,  
Serial No. 304,122

## 4 Claims. (Cl. 75—168)

The invention relates to magnesium base alloys and more particularly concerns alloys of this nature having a high degree of formability, coupled with other improved physical properties, such as high tensile and yield strengths.

Magnesium alloys are being widely used in the structural arts where a light weight metal is highly desirable, such as for use in making large castings, forgings, and the like. However, the use of these alloys in the rolled form to make sheet metal articles requiring forming operations, such as bending, drawing, and the like, has not progressed as rapidly due to the fact that, in general, alloys of good formability, permitting relatively sharp bends to be made without the article developing external cracks, usually have inferior characteristics as regards their tensile and yield strengths.

It is, accordingly, the principal object of the

sile strength and greatly increased yield strength is found in those alloys containing from between about 0.1 to 0.3 per cent of calcium and from 2 to 6 per cent of copper. The alloys containing higher percentages of alloying ingredients, such as between from 0.3 to 1 per cent of calcium and from 6 to 10 per cent of copper, while still having good ductility, have exceptionally high yield and tensile properties, and thus are especially suitable for use in casting as well as forming operations.

The following table, listing some of the properties of rolled sheet metal made from our new ternary alloys and comparing these properties with those of related binary alloys, illustrates the improvement in yield strength, tensile strength, ductility or formability, as represented by the per cent increase in elongation, of our new alloy over that of the closely related binary alloys.

Table

| 20 | Nominal composition in percent (magnesium=remainder) |      | Annealed |        |                                | Cold rolled                      |                                |                                | 20 |
|----|------------------------------------------------------|------|----------|--------|--------------------------------|----------------------------------|--------------------------------|--------------------------------|----|
|    |                                                      |      | Ca       | Cu     | Yield strength in lbs./sq. in. | Tensile strength in lbs./sq. in. | Percent elongation in 2 inches | Yield strength in lbs./sq. in. |    |
| 25 | 0.3                                                  | —    | 17,000   | 30,000 | 13                             | 27,000                           | 32,000                         | 2                              | 25 |
| 30 | —                                                    | 1.0  | 18,000   | 32,000 | 7                              | 26,000                           | 33,000                         | 2                              | 30 |
| —  | 0.3                                                  | 1.0  | 19,000   | 32,000 | 16                             | 33,000                           | 39,000                         | 3                              | —  |
| —  | 3.1                                                  | —    | 23,000   | 31,000 | 2                              | 27,000                           | 34,000                         | 2                              | —  |
| —  | 0.3                                                  | 3.2  | 22,000   | 34,000 | 13                             | 35,000                           | 41,000                         | 2                              | —  |
| —  | —                                                    | 6.0  | 24,000   | 34,000 | 3                              | 29,000                           | 36,000                         | 2                              | —  |
| —  | 0.3                                                  | 6.0  | 22,000   | 34,000 | 10                             | 35,000                           | 41,000                         | 4                              | —  |
| —  | —                                                    | 10.0 | 28,000   | 31,000 | 1                              | —                                | —                              | —                              | —  |
| 35 | —                                                    | 0.3  | 10.0     | 28,000 | 31,000                         | —                                | —                              | —                              | —  |
| —  | —                                                    | 10.0 | 24,000   | 35,000 | 9                              | 41,000                           | 46,000                         | 3                              | 35 |

invention to provide a magnesium base alloy which can be made into rolled sheet or the like, possessing a sufficient degree of ductility or formability at ordinary temperatures to be sharply bent, drawn, or otherwise shaped, while having high tensile and yield strengths.

Other objects and advantages will be apparent as the description of the invention proceeds.

Our invention resides in the discovery that a magnesium base alloy composed of from about 0.05 to 1.0 per cent of calcium and from 0.5 to 12 per cent of copper, the balance being substantially all magnesium, is endowed with the aforementioned properties. While the property of excellent formability or ductility coupled with high tensile strength and yield strength is manifest over the entire range of composition indicated, we have found that in general the preferred combination of properties, such as the most desirable ductility coupled with high ten-

25  
30  
35  
40  
45  
50

The properties listed in the above table under the section headed by the term annealed were obtained by first rolling the alloys at a temperature between about 600° to 800° F., and thereafter annealing them at various temperatures through a temperature range of from 400° to 800° F. The properties selected for the table were those of the annealed specimens which exhibited the maximum elongation. The properties listed under the section headed cold rolled were obtained by subjecting specimens of the alloys which had been hot rolled at a temperature of from 600° to 800° F. to additional rolling in the cold state to bring about a total reduction of from 2 to 10 per cent. The properties selected for the table were those of the cold rolled specimens which showed the greatest tensile and yield strengths, while having at least a 1 per cent elongation in 2 inches.

By comparison of the properties listed in the

above table, it will be observed that the combined properties of our new ternary alloys are always superior to those of the known binary alloys having similar percentages of alloying ingredients. For example, it will be noted that in the lower percentages of alloying ingredients, the cold rolled specimen of the new ternary alloy exhibited better tensile and yield strengths and an improved elongation over that of the related binary alloys. Similarly, in the higher percentages of alloying ingredients, the properties of the new ternary alloys show improvement over those of the related binary alloys.

While the new alloy is most useful in wrought form, such as sheets, due to its formability characteristics, it may also be suitably used in making castings, forgings, extruded forms, and the like.

The new alloy may be compounded in any of the ways known to the art, such as by adding the alloying ingredients to molten magnesium under suitable flux. The flux should be substantially free from magnesium chloride if the calcium content of the alloy is to be above 0.3 per cent. In those instances where an alloy is

to be compounded containing less than 0.3 per cent of calcium, magnesium chloride may be present in the flux, but in this case it is usually preferable to add the calcium last and without too much stirring to prevent the loss of calcium into the flux.

We claim:

1. A magnesium base alloy containing from 0.05 to 1 per cent of calcium and from 0.5 to 12 per cent of copper, the balance being magnesium. 10

2. A magnesium base alloy containing from 0.5 to 1 per cent of calcium and from 1.0 to 12 per cent of copper, the balance being magnesium. 15

3. A magnesium base alloy containing from 0.1 to 0.3 per cent of calcium and from 2 to 6 per cent of copper, the balance being magnesium.

4. A magnesium base alloy containing from 0.3 to 0.8 per cent of calcium and from 6 to 10 per cent of copper, the balance being magnesium. 20

JOSEPH D. HANAWALT.

JOHN C. McDONALD.

25